

1

2,928,785

**CATALYST AND HYDROCARBON CONVERSION THEREWITH**

Alfred E. Hirschler, Springfield, Pa., assignor to Sun Oil Company, Philadelphia, Pa., a corporation of New Jersey

No Drawing. Application June 14, 1955  
Serial No. 515,551

3 Claims. (Cl. 208—117)

This invention relates to catalytic compositions effective in catalytic processes for converting hydrocarbons. More particularly, this invention relates to new and improved catalytic compositions, their preparation, and to a process for converting hydrocarbons employing the new catalysts wherein a specific hydrocarbon fraction, boiling above the gasoline range, is converted to gasoline of high octane rating.

The conversion of various petroleum hydrocarbon fractions by processes such as cracking, reforming, hydro-forming, and the like, using a variety of catalysts and reaction conditions, has been described. Cracking reactions, for example, using a catalyst composed of silica and alumina which has been treated with hydrogen fluoride have been described. Such heretofore described processes, however, are not suitable for converting the hydrocarbon fraction boiling substantially within the range of from about 375° F. to 500° F. to high octane gasoline in a single stage. Instead of achieving a good yield of high octane gasoline, there is produced relatively large quantities of undesired products such as normally gaseous hydrocarbons, and the reduction of catalyst activity is rapid. It has heretofore been necessary to employ at least two stages to convert a petroleum hydrocarbon fraction boiling above the gasoline range, especially a fraction boiling within the range of from about 375° F. to 500° F., to high octane gasoline. Such processes usually involve a cracking stage wherein a portion of the hydrocarbons are converted to hydrocarbons boiling in the gasoline range, and a reforming, or hydroforming, stage to upgrade the octane rating of the gasoline. In the upgrading stage, the use of two catalysts in separate reactors with a hydrocarbon separation step between the reactors, or the use of two catalysts in a single reactor, has heretofore been required.

An object of this invention is to provide new and improved catalytic compositions effective for converting hydrocarbons.

Another object is to provide a process for converting a hydrocarbon fraction boiling within the range of from about 375° F. to 500° F. to high octane gasoline in a single stage and in good yield.

A still further object is to provide a process for the preparation of new and improved catalysts.

Other objects and their achievement, in accordance with the invention will be apparent from the following specification.

**General**

A new catalytic composition has been discovered which gives improved results in converting hydrocarbons. The new catalytic composition is a siliceous cracking catalyst, such as a natural clay or a synthetic composition containing silica and a promoter therefor. Before use the siliceous catalyst is treated with hydrogen fluoride and thereafter is leached with an aqueous solution of a water soluble salt of a promoter. When the siliceous catalyst is clay, it is preferred to use an aqueous solution of a

2

water soluble aluminum compound, and when the siliceous catalyst is a synthetic silica-promoter composition it is preferred to use an aqueous solution of a water soluble compound of the promoter, as hereinafter described. The leached composition is dried and calcined to produce a catalyst in accordance with the invention. It has been found that the resulting new catalytic composition is especially effective in converting relatively high boiling petroleum fractions, e.g., a fraction boiling within the range of from about 375° F. to 500° F., to gasoline hydrocarbons of high octane number, and that coke formation in the process is reduced to substantially a negligible value as compared to heretofore described processes.

15 The reactions involved in the process of the invention are primarily the cracking of the relatively high molecular weight hydrocarbons to hydrocarbons boiling in the gasoline range, and the dehydrogenation of hydrocarbons to produce hydrocarbons of higher octane number, such as the dehydrogenation of naphthenes to produce aromatic hydrocarbons. Hence, the process of the present invention is conveniently designated herein as "dehydro-cracking." Other reactions, however, are involved and assist in producing the high octane hydrocarbons prepared by the process, such as the isomerization of paraffins to produce more highly branched chain paraffins of relatively high octane number, and cyclization followed by dehydrogenation to produce aromatics from paraffins. A new method for catalyst preparation has been discovered which gives an especially effective catalyst in accordance with the invention. This new method of preparation is described hereinafter.

**The catalyst**

35 The catalytic composition of the invention consists essentially of a siliceous cracking catalyst, such as a natural clay or a composite of silica and a promoter therefor such as alumina, which has been treated with hydrogen fluoride and subsequently with an aqueous solution of a water soluble salt of a promoter, dried and calcined. For convenience, a silica-alumina catalyst is hereinafter used to illustrate the invention which, however, is limited only as herein defined.

45 To illustrate the preparation of a catalytic composition of the invention, a silica-alumina cracking catalyst is contacted with an aqueous solution of hydrogen fluoride. Methyl alcohol or ethyl alcohol can be substituted in whole or in part for the water in preparing this solution. The quantity of hydrogen fluoride is advantageously about 10% by weight of the silica-alumina. It is preferred to use a quantity of solution such that drainage of excess solution is not necessary, i.e., a quantity that is substantially completely adsorbed by the silica-alumina. This procedure prevents the removal by leaching of any appreciable quantity of the components of the original siliceous catalyst. However, use of a quantity of solution sufficient to require a small amount of drainage does not deleteriously affect the final catalyst. The resulting composition is then drained of excess solution, if necessary, and leached with an aqueous solution of a water soluble aluminum compound, such as aluminum nitrate. An alcohol can be substituted in whole or in part for the water, so long as the aluminum compound is soluble therein. The amount of aluminum compound is preferably at least the stoichiometric amount required to combine with the hydrogen fluoride used, and the amount of solution used is preferably sufficient to obtain substantial drainage thereof from the solid composition. After leaching with the aqueous solution of the aluminum compound, the treated silica-alumina is drained, dried and calcined. Preferably the calcining is performed with

the composition in contact with an oxygen-containing gas such as air, but an inert atmosphere can be used in this step with good results in some instances.

The preparation of the catalyst of the invention is preformed so that the leaching step immediately follows the treatment with hydrogen fluoride, i.e., the hydrogen fluoride treated composition, prior to the leaching step, is not heated to an elevated temperature or contacted with a base, since such operation does not yield a catalytic composition having an activity comparable to the activity 10 of the catalyst of the invention.

The final composition consists essentially of the original siliceous material, which is silica and alumina in the above illustration, but may contain small quantities of fluorine. It is not known why the final composition gives remarkably enhanced results as compared to the original silica-alumina composition, and as compared to the silica-alumina composition treated with hydrogen fluoride without subsequently leaching with an aqueous solution of an aluminum compound. It is believed, however, that the treatment with hydrogen fluoride in some way disrupts the crystal structure of the original siliceous composition, such as by loosening silicon atoms (such as by forming  $\text{SiF}_4$ ), and by replacing such silicon atom with aluminum atoms. Each aluminum atom which replaces a silicon atom in the lattice is believed to form an active cracking center. By contrast, in known commercial cracking catalysts, the number of active cracking sites is only a few percent or less of the total number of aluminum atoms present in the composition. The replacing of the silicon atom with an aluminum atom appears to result in highly active centers which, although probably few in number, exert a remarkably large effect upon the catalytic activity of the composition. It is known, as shown hereinafter by example, that fluorine is substantially removed by the leaching step, and that the quantity of alumina added to the composition is so small as to be practically negligible when measured as weight percent.

Synthetic silica-alumina compositions useful in preparing the composition of the present invention are well known as cracking catalysts, and heretofore described methods for their preparation may be employed in preparing the silica-alumina portion of the present catalyst. For example, the silica-alumina portion of the catalyst may be prepared by impregnating silica with aluminum salts, by directly combining precipitated hydrated alumina and silica, or by joint precipitation of alumina and silica from aqueous solutions of their salts, and by washing, drying, and heating the resulting composition. The resulting silica-alumina composition usually will have an activity index of at least 30, and preferably from 40 to 50. "Activity index," as used herein, is a measure of the efficiency of a catalyst for cracking hydrocarbons and is determined by a method described by Alexander, Proceedings Am. Pet. Inst. 27 (III) 51 (November 1947). However, silica-alumina compositions having lower activity indices can be used to prepare the catalyst of the invention for use in certain applications as hereinafter described. While the usual silica-alumina catalysts contain from about 10% to 25% alumina, useful results are obtained in accordance with the invention with silica-alumina compositions containing from 2% to 98% alumina. The silica-alumina composition can be in any desired size or shape, such as granules of irregular size or pellets of uniform size formed by known methods such as pelleting, extrusion or molding.

The silica-alumina composition, preferably after calcining, is treated with hydrogen fluoride. In some instances the hydrogen fluoride treatment, and the subsequent leaching step, can advantageously be performed without prior calcining of the silica-alumina. The quantity of hydrogen fluoride used should be between 1% and 20% by weight of the silica-alumina composition. The treatment is advantageously performed by admixing 75

the silica-alumina with an aqueous solution of hydrogen fluoride, such as by adding the aqueous solution to the silica-alumina with agitation. The amount of the solution used is preferably not in excess of the amount required to wet the silica-alumina, so that it is unnecessary to drain excess solution therefrom, but some excess with drainage does not appear deleterious. The treatment may be performed in one or more steps, but the total amount of hydrogen fluoride used, exclusive of water, should be from 1% to 20% by weight of the silica-alumina. If desired, anhydrous hydrogen fluoride, in gaseous or liquid phase, can be used to treat the silica-alumina. The period of time used for the treatment with hydrogen fluoride does not appear critical, but will usually be from 15 minutes to 24 hours, but longer times are not deleterious.

After treatment with hydrogen fluoride, the silica-alumina composition is leached with an aqueous solution of a water soluble aluminum compound. Inorganic salts 20 of aluminum such as aluminum nitrate, aluminum sulfate and aluminum chloride form suitable aqueous solutions. Aluminum nitrate is the preferred inorganic salt to use. The quantity of solution used does not appear to be critical but must be at least enough to obtain uniform 25 leaching of the silica-alumina composition. The concentration of the aluminum compound in the solution is preferably enough to supply a quantity of aluminum equivalent to the fluorine added by the hydrogen fluoride (calculated as aluminum trifluoride), i.e. a stoichiometric 30 quantity of aluminum is employed. A larger quantity is advantageous in some instances, such as where substantially complete removal of fluorine from the silica-alumina is desired, in which case from 2 to about 10 times the stoichiometrically required amount, or even 35 more, can advantageously be used. However, in some instances as little as  $\frac{1}{4}$  of the stoichiometrically required amount can be used and good results obtained, such as where a minor quantity of fluorine in the final catalytic composition is desired. In any event, the quantity of the 40 aluminum compound must be not less than this latter amount, namely, not less than enough to supply  $\frac{1}{4}$  of the quantity of aluminum stoichiometrically equivalent to the fluorine supplied by the hydrogen fluoride.

The leaching step can be conveniently performed by 45 passing the aqueous solution of an aluminum compound over the hydrogen fluoride treated silica-alumina contained in a vertical tube, the solution being passed either upwardly or downwardly through the tube. This method can be performed with a single step or with a plurality of 50 steps, depending on the quantity of solution used and the concentration of the aluminum compound in the solution. If desired, leaching can be accomplished by thoroughly admixing the hydrogen fluoride treated silica-alumina with an excess of the aqueous solution, and draining the 55 excess solution from the silica-alumina.

After the leaching step, any excess solution is drained, and the resulting composition calcined in the presence of an oxygen-containing gas. If desired, the drained composition can be washed with water prior to calcining 60 to remove any excess of the soluble aluminum compound. Advantageously the drained composition is dried prior to calcining, such as by mild heating. Calcining is advantageously performed by heating the leached silica-alumina to a temperature of about 800° F. to 65 1200° F. in the presence of air for from about 15 minutes to 6 hours. The composition from the calcining step is the catalyst of the present invention and can be used in promoting hydrocarbon reactions without further treatment.

70 It is characteristic of the present invention that the catalyst preparation does not add a significant quantity of alumina to the catalyst, the actual amount added being less than 1% by weight under any circumstances, and is usually less than 0.5% by weight. It is also characteristic, that the fluorine content of the final composition is.

usually negligible, say less than 1% by weight, but a small quantity can be permitted to remain on the catalyst if desired, as above described. The fluorine content of the final catalyst should always be less than 2% by weight to obtain good results in accordance with the present invention.

Natural siliceous clays can be substituted for the silica-alumina cracking catalyst as above described, and the resulting catalytic compositions form a preferred embodiment of the invention. Suitable clays include, for example, the hydrated silicates of aluminum, and may include hydrated silicates of other metals such as iron or magnesium or combinations thereof, such as kaolin, fuller's earth, attapulgite and the montmorillonite clays including bentonite. In this embodiment, it is preferred to use, after the treatment with hydrogen fluoride, an aqueous solution of a water soluble aluminum compound for leaching substantially as described for the silica-alumina composition.

#### Dehydrocracking

The reactions involved in the present process for converting relatively high boiling petroleum hydrocarbons to gasoline hydrocarbons of high octane rating are primarily dehydrogenation and cracking, and hence the overall process is conveniently designated as "dehydrocracking." The gasoline product preferably contains only hydrocarbons having a molecular weight lower than the hydrocarbons of the charge stock, and hence includes only the hydrocarbons which have been cracked in the process.

As above stated, the new catalytic compositions of the invention are especially suitable for dehydrocracking hydrocarbon fractions boiling in the range of from 375° F. to 500° F. to gasoline hydrocarbons of high octane rating, heretofore described processes and catalysts being unsuitable for this conversion. Accordingly, the use of the present catalyst will be described in terms of this preferred embodiment.

Especially suitable charge stocks are straight-run fractions having a naphthene content of at least 10%, and preferably above 30%, say from about 30% to 75% by volume. Other fractions such as those obtained from catalytic cracking, and recycle gas oils in general, may be used.

In the process, temperatures within the range of from 450° C. to 540° C. give good results and with the preferred hydrocarbon charge stock must be observed in order to obtain suitable conversion without excessive coke formation. The pressure is preferably maintained at about atmospheric pressure, but superatmospheric pressure up to about 100 p.s.i.g. can be used if desired. The space velocity must be maintained within the range of from about 0.5 to 3. It is preferred to employ a space velocity of from 0.8 to 1.5 since within this range there is obtained a high gasoline yield of high octane number. By "space velocity," as used herein, is meant the liquid hourly space velocity, which is the liquid volume of hydrocarbons charged per volume of catalyst per hour.

In carrying out the process of the invention, it is preferred to pass the hydrocarbon charge through a bed of catalyst under the above conditions. By such operation the activity of the catalyst is gradually decreased, principally due to the deposition of carbonaceous materials thereon. Periodic regeneration of the catalyst, such as by discontinuing the operation, flushing the catalyst bed with an inert gas such as steam, flue gas, nitrogen, or the like, and burning off the carbonaceous materials by passing an oxygen containing gas, such as air, through the hot catalyst bed, is advantageously employed. When such treatment fails to restore sufficient activity to the catalyst, regeneration as described with the additional steps of treating with hydrogen fluoride, leaching with an aqueous solution of a water soluble

compound of a metal from the II, III and IV groups of the periodic system, and calcining substantially as described for the initial catalyst preparation restores the activity of the catalyst to substantially its initial activity.

Hydrogen preferably is not employed in the process, but a small partial pressure thereof is not deleterious. In some other uses of the present catalyst, however, an atmosphere of hydrogen is advantageous, especially where operation is at superatmospheric pressure, as hereinafter described.

#### Examples

In order to illustrate a preferred catalytic composition of the invention and its use in dehydrocracking, a catalytic composition, in accordance with the invention, was prepared as follows, in which "parts" refers to parts by weight:

600 parts of a natural siliceous clay having an alumina content of about 40% by weight (calculated as  $Al_2O_3$ ) was admixed with 670 parts of ethyl alcohol and 125 15 parts of an aqueous hydrogen fluoride solution containing 60 parts hydrogen fluoride. The admixture, after standing 20 hours at room temperature, was drained and then divided into two equal parts, designated as "part A" and "part B."

20 Part A was dried and calcined in contact with air at 1000° F. for 3 hours. The resulting composition contained 6.6% by weight fluorine and is hereafter designated as catalyst A.

Part B was leached with a solution of 154 parts of 25 aluminum nitrate ( $Al(NO_3)_3 \cdot 9H_2O$ ) in 2000 parts of water by passing the solution down through a vertical tube containing the hydrogen fluoride treated clay. About 98.4% of the volume of the aqueous solution was recovered, the recovered aqueous solution containing substantially all of the fluorine originally introduced as aqueous hydrogen fluoride. The quantity of retained aluminum nitrate was sufficient to add not more than 0.36% by weight alumina to the clay. After draining, the leached composition was dried by mild heat and then calcined at about 1000° F. for about 3 hours in contact with air. The resulting catalyst contained 0.49% by weight fluorine and is hereafter designated as catalyst B.

Both catalyst A and catalyst B were used to dehydrocrack the same relatively high boiling petroleum fraction.

30 The petroleum fraction had a boiling range of from about 375° F. to 460° F., an aromatic content of about 13% by volume and a naphthene content of about 50% by volume. The following conditions were employed during the contacting: temperature of catalyst=508° C., 35 space velocity=1.01 to 1.02, pressure=atmospheric. The catalyst bed was regenerated after operation for 20 minutes by burning carbonaceous materials therefrom with a stream of air as above described. The results presented below were obtained on products collected over at least 7 cycles of catalyst regeneration. The results obtained were as follows:

|                                                   | Catalyst A | Catalyst B |
|---------------------------------------------------|------------|------------|
| 60 Products:                                      |            |            |
| Dry gas (wt. percent)                             | 6.0        | 6.9        |
| Hydrocarbons of 4 carbon atoms (wt. percent)      | 18.4       | 14.9       |
| Gasoline (C <sub>8</sub> -350° F.) (vol. percent) | 27.9       | 31.4       |
| Bottoms (vol. percent)                            | 49.3       | 46.5       |
| Coke (wt. percent)                                | 2.3        | 4.45       |
| Octane rating of gasoline                         | 97.0       | 97.7       |
| Liquid recovery (vol. percent)                    | 95.6       | 92.8       |
| Conversion (vol. percent)                         | 50.7       | 53.5       |

65 The foregoing data show not only an increase in the total conversion but an even greater increase in the quantity of gasoline formed, thus showing the catalyst of the invention to give high selectivity for the production of gasoline from high boiling hydrocarbons.

70 To further illustrate the catalysts of the invention using a synthetic siliceous cracking catalyst, a synthetic silica-alumina cracking catalyst prepared by coprecipitation,

containing about 13% by weight  $\text{Al}_2\text{O}_3$  and about 87% by weight  $\text{SiO}_2$ , and having an activity index of about 46, was treated with hydrogen fluoride. 511 parts of the synthetic silica-alumina in the form of pellets was treated with about 37 parts of hydrogen fluoride dissolved in a mixture of about 570 parts of ethyl alcohol and 38 parts of water by contacting for 16 hours. The treated pellets were introduced into a vertically positioned column and leached for 1 hour with a quantity of an aqueous solution containing 185.9 parts of aluminum nitrate nonylhydrate per 814.1 parts of water to cover the pellets. The solution was drained and a fresh portion of the same aqueous solution percolated downwardly through the pellets, about 1000 parts of the solution being used.

The leached composition was drained, dried under infra-red heat at about  $240^\circ \text{ F.}$ , and then calcined for about 2.5 hours at a temperature of from about  $1000^\circ \text{ F.}$  to  $1200^\circ \text{ F.}$  in contact with air.

The resulting composition consisted essentially of about 13% by weight  $\text{Al}_2\text{O}_3$  and 87% by weight  $\text{SiO}_2$ , with a minor quantity, less than about 1% of fluorine. The so-formed catalytic composition, when used to convert hydrocarbons, gives good results in accordance with the process of the invention.

When other natural clays or synthetic siliceous compositions are employed, results substantially equivalent to those above described are obtained, but with such compositions containing a smaller percentage of alumina, the selectivity for the production of gasoline appears to be even greater than shown by the foregoing data.

The catalyst of the invention can be used in other reactions involving the conversion of hydrocarbons, such as the catalytic cracking of gas oils, destructive hydrogenation using elevated pressures in an atmosphere of hydrogen, reforming, and the like, in which catalytic conversion conditions known to be effective in such processes give good results.

The invention claimed is:

1. A new composition of matter effective for converting hydrocarbons prepared by contacting a natural clay cracking catalyst with from 1% to 20% by weight hydrogen fluoride, leaching the resulting composition with an aqueous solution of a water soluble aluminum compound wherein the quantity of said aluminum compound is at least  $\frac{1}{4}$  the stoichiometric quantity required to form aluminum trifluoride by reaction of said hydrogen fluoride and said aluminum compound the volume of the

solution being sufficiently great to reduce by leaching the fluorine content of the composition to less than about 1%, and calcining the leached composition in contact with an oxygen containing gas.

- 5 2. A new composition of matter effective for converting hydrocarbons prepared by contacting a natural clay cracking catalyst with from 1% to 20% by weight of hydrogen fluoride, leaching the resultant composition with an aqueous solution of a heat decomposable aluminum salt, the amount of salt in the solution being sufficient to deposit on the composition a small amount, but less than one percent of the composition, of the salt, the total volume of the solution being sufficiently great to reduce by leaching the fluorine content of the composition to less than about one percent, and calcining the leached composition in contact with an oxygen-containing gas.
- 10 3. Process for the conversion of a hydrocarbon fraction boiling in the range of from about  $375^\circ \text{ F.}$  to  $500^\circ \text{ F.}$  to gasoline hydrocarbons which comprises contacting said hydrocarbon fraction at a temperature of from  $450^\circ \text{ C.}$  to  $540^\circ \text{ C.}$ , a pressure of from atmospheric to 100 p.s.i.g. and a space velocity of from 0.5 to 3 with a catalytic composition prepared by contacting a natural clay catalyst with from 1% to 20% by weight of hydrogen fluoride, leaching the resultant composition with an aqueous solution of a heat decomposable aluminum salt, the amount of salt in the solution being sufficient to deposit on the composition a small amount, but less than one percent of the composition, of the salt, the total volume of the solution being sufficiently great to reduce by leaching the fluorine content to less than about 1%, and calcining the leached composition in contact with an oxygen-containing gas.
- 15 4. Process for the conversion of a hydrocarbon fraction boiling in the range of from about  $375^\circ \text{ F.}$  to  $500^\circ \text{ F.}$  to gasoline hydrocarbons which comprises contacting said hydrocarbon fraction at a temperature of from  $450^\circ \text{ C.}$  to  $540^\circ \text{ C.}$ , a pressure of from atmospheric to 100 p.s.i.g. and a space velocity of from 0.5 to 3 with a catalytic composition prepared by contacting a natural clay catalyst with from 1% to 20% by weight of hydrogen fluoride, leaching the resultant composition with an aqueous solution of a heat decomposable aluminum salt, the amount of salt in the solution being sufficient to deposit on the composition a small amount, but less than one percent of the composition, of the salt, the total volume of the solution being sufficiently great to reduce by leaching the fluorine content to less than about 1%, and calcining the leached composition in contact with an oxygen-containing gas.
- 20 5. Process for the conversion of a hydrocarbon fraction boiling in the range of from about  $375^\circ \text{ F.}$  to  $500^\circ \text{ F.}$  to gasoline hydrocarbons which comprises contacting said hydrocarbon fraction at a temperature of from  $450^\circ \text{ C.}$  to  $540^\circ \text{ C.}$ , a pressure of from atmospheric to 100 p.s.i.g. and a space velocity of from 0.5 to 3 with a catalytic composition prepared by contacting a natural clay catalyst with from 1% to 20% by weight of hydrogen fluoride, leaching the resultant composition with an aqueous solution of a heat decomposable aluminum salt, the amount of salt in the solution being sufficient to deposit on the composition a small amount, but less than one percent of the composition, of the salt, the total volume of the solution being sufficiently great to reduce by leaching the fluorine content to less than about 1%, and calcining the leached composition in contact with an oxygen-containing gas.
- 25 6. Process for the conversion of a hydrocarbon fraction boiling in the range of from about  $375^\circ \text{ F.}$  to  $500^\circ \text{ F.}$  to gasoline hydrocarbons which comprises contacting said hydrocarbon fraction at a temperature of from  $450^\circ \text{ C.}$  to  $540^\circ \text{ C.}$ , a pressure of from atmospheric to 100 p.s.i.g. and a space velocity of from 0.5 to 3 with a catalytic composition prepared by contacting a natural clay catalyst with from 1% to 20% by weight of hydrogen fluoride, leaching the resultant composition with an aqueous solution of a heat decomposable aluminum salt, the amount of salt in the solution being sufficient to deposit on the composition a small amount, but less than one percent of the composition, of the salt, the total volume of the solution being sufficiently great to reduce by leaching the fluorine content to less than about 1%, and calcining the leached composition in contact with an oxygen-containing gas.
- 30 7. Process for the conversion of a hydrocarbon fraction boiling in the range of from about  $375^\circ \text{ F.}$  to  $500^\circ \text{ F.}$  to gasoline hydrocarbons which comprises contacting said hydrocarbon fraction at a temperature of from  $450^\circ \text{ C.}$  to  $540^\circ \text{ C.}$ , a pressure of from atmospheric to 100 p.s.i.g. and a space velocity of from 0.5 to 3 with a catalytic composition prepared by contacting a natural clay catalyst with from 1% to 20% by weight of hydrogen fluoride, leaching the resultant composition with an aqueous solution of a heat decomposable aluminum salt, the amount of salt in the solution being sufficient to deposit on the composition a small amount, but less than one percent of the composition, of the salt, the total volume of the solution being sufficiently great to reduce by leaching the fluorine content to less than about 1%, and calcining the leached composition in contact with an oxygen-containing gas.
- 35

References Cited in the file of this patent

UNITED STATES PATENTS

|              |               |       |                |
|--------------|---------------|-------|----------------|
| 2,154,527    | Pier          | ----- | Apr. 18, 1939  |
| 2,245,157    | Pier et al.   | ----- | June 10, 1941  |
| 2,340,698    | Ruthruff      | ----- | Feb. 1, 1944   |
| 2,356,303    | Connolly      | ----- | Aug. 22, 1944  |
| 2,371,890    | Herold et al. | ----- | Mar. 20, 1945  |
| 2,400,020    | Pierce        | ----- | May 7, 1946    |
| 40 2,450,394 | Brown et al.  | ----- | Sept. 28, 1948 |
| 45 2,506,923 | Hoekstra      | ----- | May 9, 1950    |